

## UNITED STATES PATENT OFFICE

CHARLES VANGREVENYNGE, OF LA CELLE-ST. CLOUD, AND HENRY ELION, OF PARIS,  
FRANCE

## METAL ALLOY

No Drawing. Application filed August 28, 1930, Serial No. 478,560, and in France January 7, 1930.

This invention relates to light alloys of aluminum, in which copper, nickel, magnesium, and chromium act as additional constituents to the aluminum and to the impurities contained therein, such as iron, silicium and alumina.

5 The complex alloys are characterized first by their very high breaking load R, their high coefficient of expansion A, as well as 10 by their apparent limit of elasticity E.

Second, that which differentiates them from alloys hitherto known, for example those with a base of aluminum, copper, magnesium and manganese, is that by reason of 15 the presence of nickel their great facility of transformation allows of forging, swaging, rolling and wire-drawing with the greatest ease and without waste to the extent which occurs with alloys hitherto known.

20 Within the scope of this invention, a wide range of alloys can be obtained according to the proportions of the constituent elements of the alloy.

An alloy found excellent under test is obtained according to the following composition:

|           | Per cent |
|-----------|----------|
| Aluminum  | 94.85    |
| Copper    | 3.40     |
| 30 Nickel | 0.50     |
| Chromium  | 0.50     |
| Magnesium | 0.75     |

The proportions of the constituents may 35 also be as follows:

|              | Per cent     |
|--------------|--------------|
| Copper       | 1.50 to 5.00 |
| Nickel       | 0.25 to 2.50 |
| Chromium     | 0.25 to 1.50 |
| 40 Magnesium | 0.25 to 2.00 |

In the manufacture of these alloys there is first formed a basic alloy containing all the additional constituents Cu, Ni, Cr, excepting the magnesium, this basic alloy being introduced into the aluminum bath to be treated in suitable proportion.

The order of mixing the constituents for the basic alloy is immaterial, it being only 50 essential that the successive temperatures

necessary for the introduction of each of the constituents shall be such as to give a perfect mixture.

Instead of using a basic alloy, the alloy sought can be found by employing binary 55 alloys of each of the additional metals, that is to say alumino-copper, alumino-nickel, alumino-chromium.

The magnesium is introduced at the end of the operation before casting, either in the 60 state of pure metal or in the state of binary alloy, alumino-magnesium, to avoid losses or recovering of the metal.

Commercial aluminum of 98%-99% purity can be employed, that is to say, aluminum 65 in which the total of iron and silicium is less than 2%, the silicium being about 0.4%.

Better results may be obtained by using an aluminum of 99%-99.5% purity, that is, 70 second class aluminum, containing the minimum percentage of iron.

A light alloy having the composition defined above and obtained with a 98%-99% aluminum will give average characteristics 75 superior to those of the usual alloys.

These characteristics may be much improved by subjecting the alloy to an appropriate thermic treatment consisting, as known, in reheating in a salt bath at about 500° C. (475-500° C.), composed of sodium 80 nitrate and potassium nitrate, followed by a water bath and an aging, or more exactly a ripening, from 8 to 10 days.

Under such conditions, there have been 85 found, during mechanical tests effected with samples of metal thus treated, forged, swaged or rolled, the average characteristics of:

|                           |       |
|---------------------------|-------|
| Apparent elastic limit    | E=27  |
| Breaking strain           | R=45  |
| Coefficient of elongation | A=20% |

It should be particularly noted that the role of the nickel is to give to the alloy its greatest facility of transformation without danger of waste, and to enable it to be drawn into wire with the greatest facility.

It is obvious, moreover, that modifications of detail may be made within the scope of the invention and in particular the proportion 100

of the constituents may vary according to whether the metal is to be used molten, or to be swaged or rolled.

5 This same metal run into chills gives in the rough chilled casting and without any treatment, the average characteristics as follows:

Apparent elastic limit..... E=14 to 16  
 10 Breaking strain..... R=19 to 24  
 Coefficient of elongation... A= 5 to 8%

What we claim is:

1. An aluminium alloy consisting of 94.85% aluminium, 3.40% copper, 0.50% nickel, 0.50% chromium and 0.75% magnesium.
- 15 2. A light aluminium alloy, consisting of aluminium, copper, nickel, magnesium and chromium and containing of:

|                | Per cent     |
|----------------|--------------|
| Copper .....   | 1.50 to 5.00 |
| Nickel .....   | 0.25 to 2.50 |
| Chromium ..... | 0.25 to 1.50 |
| Magnesium..... | 0.25 to 2.00 |

In witness whereof they affix their signatures.

CHARLES VANGREVENYNGE.  
 HENRY ELION.

30

35

40

45

50

55

60

65